

## UNITED STATES PATENT OFFICE

2,396,129

PLASTICIZERS AND METHOD OF MAKING  
THE SAMEErnest A. Rodman, Newburgh, N. Y., assignor to  
E. I. du Pont de Nemours & Company, Wilming-  
ton, Del., a corporation of DelawareNo Drawing. Application March 25, 1942,  
Serial No. 436,157

15-Claims. (Cl. 106—171)

This invention relates to new and novel plasticizers for cellulose derivatives and methods of making the same.

At present certain vegetable oils are used very extensively as plasticizers for cellulose derivatives, particularly cellulose nitrate. Among the more common examples are castor oil, cottonseed oil, rapeseed oil, etc. While these vegetable oils are satisfactory for plasticizing nitrocellulose coatings in a great many uses, they cannot be used where the coating is to be subjected to elevated temperatures, since the oil will spew to the surface when subjected to temperatures of approximately 160° F. and higher. For this reason the vegetable oils are not entirely satisfactory as plasticizers for cellulose nitrate coatings.

The plasticizers herein disclosed are of particular value with cellulose derivatives for coating fabrics used extensively as a bookbinding material because of their superior wear resistance, vermin resistance, washability and easily fabricating qualities. When cellulose nitrate coatings are plasticized with certain plasticizers of vegetable origin, they may be objectionable because they tend to spew to the surface when subjected to elevated temperatures.

The cellulose nitrate coated fabrics are usually supplied to the bookbinders with a surface design or grain embossed in the coating which is made up into book covers by covering a stiff or semi-flexible card board with the coated fabric. It is often desired to print the front portion as well as the backbone of the book cover with a design of different color from the coating on the fabric. It is often desired to flatten out a portion of the embossed surface after the coated fabric is made up into a book cover where it is desired to print. This is accomplished by using a smooth embossing plate in a conventional embossing apparatus in which the book cover is subjected to heat and pressure to flatten out a limited area to be printed. This operation is referred to in the bookbinding industry as "blanking." The heat and pressure on the coating employed in the blanking operation causes the oil in the cellulose nitrate coating to exude or spew to the surface which interferes with the drying of the printing inks which are subsequently applied to the blanked out area. It is, therefore, necessary to allow the book covers to stand twelve to twenty-four hours after blanking in order that the oil which exudes to the surface may be reabsorbed by the coating before the covers are printed. This delay between blanking and the printing operation is very costly to the bookbinder in that it

delays production and large storage space is required for the book covers between the blanking and printing operation.

The primary object of this invention is to provide a new and novel plasticizer for nitrocellulose which will not exude or spew from a dry nitrocellulose film when subjected to elevated temperatures and pressures.

A more specific object is the provision of a plasticized cellulose nitrate composition for coating fabrics for book-binding material which may be blanked and printed immediately thereafter.

These and other objects will be readily apparent to those skilled in the art as the description of the invention proceeds.

15 The foregoing objects are accomplished by reacting certain blown oils with certain carboxylic acids or anhydrides in such manner that when the reaction product is present within certain limits in a dried cellulose nitrate coating, it is resistant to exuding to the surface when the coating is subject to the influences of heat and pressure. The reaction product of blown corn oil and phthalic or maleic acid is particularly satisfactory.

20 25 Raw corn oil is unsatisfactory as a plasticizer for nitrocellulose in that it is relatively incompatible with nitrocellulose. It has been discovered that by blowing the raw corn oil with air that a suitable product is obtained which is sufficiently compatible with nitrocellulose to effect plasticization to permit its use with nitrocellulose where flexible coatings are desired. However, if the dry films comprising the blown corn oil and nitrocellulose are subjected to temperature as high as 180° F., the oil will spew to the surface of the film and result in a sticky or tacky surface. This prohibits the use of the oxidized corn oil in coatings which are to be subjected to temperatures above 180° F., such as book-binding material which is normally blanked at temperatures well in excess of 180° F.

30 35 It has been discovered that if the blown corn oil is reacted with phthalic anhydride or similar acid anhydride, the exudation characteristics of the pyroxylin composition containing the reaction product are greatly improved, permitting the use of the reacted corn oil in compositions which are to be subjected to heat as high as 240-250° F. which are commonly encountered in the embossing and processing of nitrocellulose coated fabrics.

40 45 The detailed description hereinafter is given for the purpose of illustration and not limitation.

45 50 The preparation of oxidized corn oil phthalate comprises two steps, the first of which is the treat-

ment of the oil by blowing with air until the desired extent of reaction has taken place between the air and the oil as measured essentially by the increased viscosity of the oil. The second step comprises the reaction of the oxidized oil with phthalic anhydride. Experimentation in regard to solubility of the untreated oil and exudation characteristics of the coated products has indicated that the ultimate product containing 95 per cent of oxidized oil and 5 per cent of phthalic anhydride is most desirable.

A grade of raw corn oil which has been found to be particularly suited for the purpose of this invention has the following specifications:

|                           |          |             |
|---------------------------|----------|-------------|
| Solidifying point         | °C       | 10-15       |
| Saponification value      |          | 188-193     |
| Iodine number             |          | 113-129     |
| Saturated fatty acid      | per cent | 11.8        |
| Unsaturated fatty acid    | do       | 86.5        |
| Acetyl value              |          | 10-11.5     |
| Unsaponifiable matter     |          | 1.3-2.0     |
| Refractive index/15.5° C. |          | 1.475-1.477 |

The raw corn oil is charged to a suitable reaction vessel, i. e. fitted with a thermometer, a heating arrangement, and a sparger pipe in the bottom to disperse the air through the oil. The oil is heated to approximately 93° C. Simultaneously with the heating, air is forced through the oil.

During the process of blowing the oil it is heated to 93° C. and the blowing is continued until a viscosity of approximately 35 to 50 seconds (Gardner-Holdt tube) at 25° C. is obtained. On this scale 1.467 seconds equals one poise at 25° C. To obtain this viscosity with the oil heated to 93° C. requires approximately 40 hours.

It has been found that the extent to which the oil is oxidized by blowing with air has a considerable effect in its reactivity with phthalic anhydride, and by experimentation it has been discovered that if the raw corn oil is blown until a viscosity of 35 to 50 seconds (Gardner-Holdt tube at 25° C.) is obtained, the most satisfactory reactivity with phthalic anhydride is obtained.

If the oil is blown until a viscosity of 55 seconds (Gardner-Holdt tube at 25° C.) is obtained, the subsequent reaction with phthalic anhydride proceeds at such a rapid rate that it is very difficult to control the reaction so as to obtain a uniform product. If the blowing of the oil is stopped when the viscosity of the oil has reached 30 seconds (Gardner-Holdt tube at 25° C.) the subsequent reaction with phthalic anhydride is very slow and the resulting product is less miscible with nitrocellulose coating composition and is much darker in color. Further if the oil is only blown to 30 seconds, a greater portion of blending solvent is required for satisfactory miscibility with nitrocellulose coating compositions dispersed in the usual alcohol and ester solvent mixtures.

It has been discovered by experimentation that if the temperature of the oil during the oxidation process exceeds 105° C. a cracking and polymerization of the oil takes place and the resulting product is not sufficiently reactive with phthalic anhydride. If the temperature of the oil during the oxidizing process is approximately 80° C., the time required for blowing to obtain a viscosity of 35 to 50 seconds (Gardner-Holdt tube at 25° C.) is approximately 70 hours. The lower the temperature of the oil during the oxidizing process, the longer it is required for the blowing of the oil to obtain the optimum viscosity range of

35 to 50 seconds (Gardner-Holdt tube at 25° C.). It is not economically practical to blow the oil longer than 70 hours.

After the oil has reached 35 to 50 seconds viscosity (Gardner-Holdt tube at 25° C.) the air being forced through the oil is stopped and the temperature of the oil elevated to 132° C. During the elevation of the temperature of the oil, a mechanical stirrer is used to agitate the oil and carbon dioxide gas is slowly bubbled through the sparger pipe to facilitate agitation and to aid in preventing discoloration of the product. When the temperature of the blown oil has reached 132° C., phthalic anhydride is added slowly to the charge with vigorous agitation. For every 95 parts of oxidized corn oil five parts of phthalic anhydride are added to the reaction kettle. Since the reaction runs through to completion the reaction product has the approximate composition of 95 parts oxidized corn oil and five parts of phthalic anhydride.

During the addition of the phthalic anhydride there is an exothermic reaction and the temperature rises to 140° C. Temperature is maintained at this point until a viscosity of approximately between 200 and 250 seconds (Gardner-Holdt tube at 25° C.) is obtained. When the desired viscosity is reached, the oil is cooled as rapidly as possible to about 65° C. Sufficient solvent is added to the reaction kettle to make a 90% solution of the blown corn oil phthalate. The solvent added to the reaction kettle should be miscible with both the reaction product and pyroxylin. Butanol has been found satisfactory for this purpose, as well as toluol, pentasol and mixtures of various solvents. The material is removed from the reaction kettle and is ready for use as a nitrocellulose plasticizer for book-binding material. The butanol is added to facilitate compatibility of the oxidized corn oil phthalate in a nitrocellulose coating composition dispersed in an alcohol-ester solvent mixture, such as e. g., ethyl alcohol and ethyl acetate.

The oxidized corn oil phthalate has the following properties:

|                     |      |            |
|---------------------|------|------------|
| Viscosity at 25° C. | Sec. | 1 200-250  |
| Acid number         |      | 23-30      |
| Iodine number       |      | 65-75      |
| Saponification No   |      | 270-300    |
| Color               |      | Dark amber |

<sup>1</sup> Gardner-Holdt tube.

In the method outlined above 95 parts of the oxidized oil are reacted with 5 parts of the anhydride. However, it has been found that desirable plasticizers can be made using as much as 15 parts of the anhydride to 85 parts of the oxidized oil. Plasticizers containing more than 15 parts of the anhydride to 85 parts of oxidized oil are not entirely satisfactory because of incomplete reaction of the anhydride with the oxidized oil, which results in a material having an excessively high acid number for the purposes of this invention.

Plasticizers containing less than 2% of phthalic anhydride have not been found satisfactory for the purposes of this invention since such small modifications of the oxidized oil do not result in any material advantage.

In a like manner oxidized corn oil maleate may also be prepared in which case 97.8 parts of oxidized corn oil is reacted with 2.2 parts of maleic anhydride at a temperature of 160° C. instead of 140° C. as in the case of phthalic anhydride. Where maleic anhydride is used 2.2

parts of maleic anhydride are used in place of 5 parts of phthalic anhydride which is the reactive equivalent. The result is essentially the same except in the case of the oxidized corn oil maleate which is of a light straw color which is of extreme importance in the case of its use with light colored coating compositions. Plasticizers containing more than 5 parts of the maleic anhydride as well as those containing less than 1 part are not satisfactory for the purposes of this invention for the same reasons discussed above in connection with the preferred range of phthalic anhydride.

*Example I*

A bookbinding material referred to in the trade as an impregnated cloth as distinguished from a coated cloth is prepared as follows:

To a woven fabric sheeting running 4.75 yards per pound per 39" width there is applied three coats of the following composition by means of a sharp doctor knife:

|                                                        | Per cent |
|--------------------------------------------------------|----------|
| Cellulose nitrate                                      | 10.50    |
| 90% solution of oxidized corn oil phthalate in butanol | 14.00    |
| Pigments                                               | 17.85    |
| Butanol                                                | 15.06    |
| Ethyl acetate                                          | 21.69    |
| Ethyl alcohol                                          | 21.30    |

The method of preparing the above composition which comprises first dissolving the cellulose nitrate in the solvents and separately grinding the pigments in the blown corn oil phthalate and then combining the materials is well known in the art and further detailed description does not appear to be necessary.

The tension of the fabric and position of the doctor knife is so adjusted that the coating composition is actually driven into the interstices of fabric instead of bridging across them. Approximately 4.7 ounces of the wet coating composition are applied to the fabric which corresponds to approximately 2.0 ounces of non-volatile components. The material is passed through a heated chamber after each successive coat to expel the volatile solvents. Following the impregnating of the fabric it is embossed by conventional embossing methods, such as roller or plate embossing apparatus in which the treated fabric is subjected to a heat and pressure treatment. A design counter to the design of the embossing element is transferred to the treated fabric. At this stage the material is supplied to the bookbinder in long lengths.

The bookbinder cuts the material to the desired shape and attaches the treated fabric to a rigid or semi-rigid material to form a book cover. In order to further enhance the appearance of the book cover and provide a smooth printing surface for titles and decorative work the thus prepared cover is subjected to a blanking operation in which a limited area of the cover is flattened out by a heated smooth embossing plate under pressure. The temperature of the smooth embossing plate is approximately 280° F. and sufficient pressure is applied to flatten or obliterate the original embossed design. During this heat and pressure treatment the blown corn oil phthalate does not exude to the surface. Immediately following the blanking operation and while the blanked area is still hot it can be printed with conventional printing inks designed for use on cellulose nitrate containing surfaces without interfering with the nor-

mal drying time of the printing ink. A suitable printing ink for the cellulose nitrate treated fabric is disclosed in U. S. Patent 2,049,507, which issued August 4, 1936, to McBurney et al.

*Example II*

A coated fabric as distinguished from an impregnated fabric is prepared as follows: To a cotton sheeting running 3.69 yards per pound per 39" width is applied a plurality of coats of the following composition by means of a doctor knife:

|                                                        | Per cent |
|--------------------------------------------------------|----------|
| Cellulose nitrate                                      | 11.65    |
| Pigments                                               | 9.65     |
| 90% solution of oxidized corn oil phthalate in butanol | 21.10    |
| Butanol                                                | 14.70    |
| Ethyl acetate                                          | 21.45    |
| Ethyl alcohol                                          | 21.45    |

The doctor knife and tension of the fabric is adjusted so that the coating is applied on the surface of the fabric rather than driven into the interstices. Sufficient coats of the above composition are applied to deposit approximately ten ounces per yard of wet composition on the fabric which correspond to 4.2 ounces per yard of non-volatile components. A final surface coat of the following composition is applied in the amount of 1.5 wet ounces per yard which corresponds to 0.2 dry ounce per yard.

|                   | Percent |
|-------------------|---------|
| Cellulose nitrate | 12.35   |
| Ethyl acetate     | 43.83   |
| Ethyl alcohol     | 43.82   |

The volatile solvents are expelled after each successive coat by passing through a heated chamber. The material prepared is next embossed with an overall design by conventional embossing apparatus. The material thus prepared is supplied to the book-binders. It is ready to be made up into book covers and treated in the same manner as mentioned in Example I by blanking and printing immediately after blanking.

While the preferred embodiment of this invention employs raw corn oil having an iodine value of 113 to 129 as a starting material in the manufacturing of the oil phthalate, other unsaturated semi-drying oils having an iodine value of 80 to 135 may be used with varying degrees of success. The following oils which are listed below with the corresponding iodine value fall within the scope of this invention as equivalents of raw corn oil used to illustrate the invention.

| Oil:           | Iodine value |
|----------------|--------------|
| Raw corn       | 113-129      |
| Raw peanut     | 88-98        |
| Raw cottonseed | 103-111      |
| Raw soya bean  | 122-134      |
| Raw olive      | 79-88        |

65 Oils having an iodine value below 80 contain such quantities of saturated components which do not oxidize sufficiently when blown with air, that the blown oil will not react satisfactorily with phthalic acid to give the desired properties.

70 Oils having an iodine value greater than 135 are so highly unsaturated as to form solid oxidation products and are not satisfactory in preparing nitrocellulose plasticizers.

75 The preferred embodiment of this invention employs the anhydride of the carboxylic acid

since they are more active. It is, however, within purview of the invention to employ carboxylic acids and their anhydrides other than phthalic acid. Those which may be used to react with the oxidized oils include unsaturated dicarboxylic acids, such as, e. g., maleic acid; saturated dicarboxylic acids, such as, e. g. succinic and adipic acids; saturated monobasic carboxylic acids, such as, e. g. acetic and lauric acids; and carboxylic acids; with hydroxyl groups, such as, e. g. lactic acid.

In the claims and specification, the term "acid" is used generically to include the anhydride as well as the carboxylic acid, and in most cases the former is preferred.

This method is to be distinguished from making alkyd resins wherein they are modified with a blown oil in that the embodiments of this invention do not require the addition of a polyhydric alcohol. In the present case no glycerine 20 as such is added and the acid is present in a relatively very minor proportion.

The new plasticizers herein disclosed are useful in plasticizing certain polyvinyl resins, such as, e. g. the copolymer vinyl acetate and vinyl chloride resins disclosed in U. S. Patent 1,935,577 to Reid; the copolymer of vinyl chloride and diethyl fumarate or dimethyl fumarate resins disclosed in U. S. Patent 1,945,307 to Dykstra; and the polyvinyl acetal resins disclosed in U. S. Patent 30 Reissue 20,430 to Morrison et al. A small portion of a solvent type plasticizer is sometimes desirable to use with the new plasticizers herein disclosed when plasticizing polyvinyl resins to prevent the blown semi-drying oil-acid reaction product from sweating out.

This invention will find great utility in the nitro-cellulose lacquer industry wherever a non-spewing plasticizer is desired. The non-spewing plasticizer herein disclosed will also find great utility as a plasticizer for ethyl cellulose, as well as for synthetic resins with which it is compatible therewith. Coatings employing the non-spewing plasticizer may be applied over rigid base materials, such as wood, metal, etc., as well as flexible base materials, such as paper, cellulose film, non-woven fabrics, etc. Specific uses as a nitro-cellulose plasticizer other than book-binding material described in the foregoing examples include outdoor furniture upholstery, lacquered table cloths, and coated fabrics in general. Other important uses will be readily apparent to those skilled in the art. Cellulose derivatives, such as ethyl cellulose, benzyl cellulose, and similar film-forming cellulose derivatives may replace the cellulose nitrate.

The primary advantage of the invention is the provision of a non-spewing nitrocellulose plasticizer which permits the use of plasticized nitrocellulose compositions at temperatures which cause spewing of the conventional vegetable oil plasticizers. A further advantage is the provision of a bookbinding material which may be blanked and printed immediately over the blanked area.

It is apparent that many widely different embodiments of this invention may be made without departing from the spirit and scope thereof, and therefore, it is not intended to be limited except as indicated in the appended claims.

I claim:

1. A composition consisting of the reaction product of corn oil blown to a viscosity of 35 to 50 seconds (Gardner-Holdt Scale) and material

selected from the group consisting of phthalic acid, maleic acid, and their anhydrides.

2. The product of claim 1 in which the dicarboxylic acid is phthalic acid and the ratio of oil to phthalic acid is between 85 to 15 and 95 to 5.

3. The product of claim 1 in which the dicarboxylic acid is maleic acid and the ratio of oil to maleic acid is between 95 to 5 and 99 to 1.

4. A nitrocellulose composition comprising nitrocellulose and the reaction product of blown corn oil and material selected from the group consisting of phthalic acid, maleic acid and their anhydrides, the said corn oil having been blown to a viscosity of 35 to 50 seconds (Gardner-Holdt Scale) before reacting with the acid material.

5. A nitrocellulose composition comprising nitrocellulose and blown corn oil phthalate the corn oil having been blown to a viscosity of 35 to 50 seconds (Gardner-Holdt Scale) before reacting with phthalic acid.

6. A nitrocellulose composition comprising nitrocellulose and blown corn oil maleate the corn oil having been blown to a viscosity of 35 to 50 seconds (Gardner-Holdt Scale) before reacting with maleic acid.

7. The method of preparing a plasticizer for nitrocellulose compositions which does not spew therefrom at elevated temperatures which consists in blowing a semi-drying oil having iodine number between 80 and 135 until a viscosity of 35 to 50 seconds (Gardner-Holdt Scale) is reached and thereupon reacting the same with material selected from the group consisting of phthalic acid, maleic acid and their anhydrides.

8. Process of preparing a non-spewing nitrocellulose plasticizer comprising blowing a raw semi-drying oil until the viscosity of the oil reaches 35 to 50 seconds (Gardner-Holdt tube at 25° C.), and thereupon reacting the blown oil with phthalic anhydride until the viscosity of the reaction product reaches a viscosity of 200-250 seconds (Gardner-Holdt tube at 25° C.).

9. Process of preparing a non-spewing nitrocellulose plasticizer comprising blowing at 80-105° C. a raw corn oil until the viscosity of the oil reaches 35 to 50 seconds (Gardner-Holdt tube at 25° C.), and thereupon reacting the oxidized corn oil with phthalic anhydride until the viscosity of the reaction product reaches a viscosity of 200-250 seconds (Gardner-Holdt tube at 25° C.).

10. Process of preparing a non-spewing nitrocellulose plasticizer comprising oxidizing raw corn oil by blowing with air at 80-105° C. until the viscosity of the oxidized oil reaches 35 to 50 seconds (Gardner-Holdt tube at 25° C.) said corn oil having an iodine number between 80 and 135 seconds before oxidation, reacting the said oxidized corn oil with phthalic anhydride until the viscosity of the reaction product reaches a viscosity of 200-250 seconds (Gardner-Holdt tube at 25° C.), and adding sufficient solvent to the reaction product to make a 90 per cent solution of said reaction product.

11. The process of claim 10 in which the ratio of oil to phthalic anhydride is 95 parts of oil to 5 parts of phthalic anhydride.

12. Process of preparing a non-spewing nitrocellulose plasticizer comprising blowing a raw semi-drying oil until the viscosity of the oil reaches 35 to 50 seconds (Gardner-Holdt tube at 25° C.) and thereupon reacting the blown oil with maleic anhydride until the viscosity of the reaction product reaches a viscosity of 200-250 seconds (Gardner-Holdt tube at 25° C.).

13. Process of preparing a non-spewing nitro-cellulose plasticizer comprising blowing at 80-105° a raw corn oil until the viscosity of the oil reaches 35 to 50 seconds (Gardner-Holdt tube at 25° C.), and thereupon reacting the oxidized corn oil with maleic anhydride until the viscosity of the reaction product reaches a viscosity of 200-250 seconds (Gardner-Holdt tube at 25° C.).

14. Process of preparing a non-spewing nitro-cellulose plasticizer comprising oxidizing raw corn oil by blowing with air at 80-105° C. until the viscosity of the oxidized oil reaches 35 to 50 seconds (Gardner-Holdt tube at 25° C.) said corn

oil having an iodine number between 80 and 135 seconds before oxidation, reacting the oxidized corn oil with maleic anhydride until the viscosity of the reaction product reaches a viscosity of 200-250 seconds (Gardner-Holdt tube at 25° C.), and adding sufficient solvent to the reaction product to make a 90 per cent solution of said reaction product.

15. The process of claim 14 in which the ratio of oil to maleic anhydride is 97.8 parts of oil to 2.2 parts of maleic anhydride.

ERNEST A. RODMAN.